

Aug. 27, 1940.

V. W. DAVID

2,213,039

WATER SHUT-OFF METHOD AND COMPOSITION FOR WELLS

Filed Nov. 14, 1938



BY

*John Brown*

ATTORNEY

## UNITED STATES PATENT OFFICE

2,213,039

## WATER SHUT-OFF METHOD AND COMPOSITION FOR WELLS

Vern W. David, Bakersfield, Calif.

Application November 14, 1938, Serial No. 240,311

5 Claims. (Cl. 166—21)

This invention relates to well material, particularly to a composition of matter and the process of forming the same, and the method of its use in certain practices, as hereinafter identified.

5 The present invention in one of its aspects contemplates a composition of matter adapted to take the place of ordinary cement, such as used in oil wells, when it becomes necessary to cement off a string of casing for any reason whatsoever. 10 More particularly, the present invention may cooperate with my invention described in a copending application entitled "Formation sealing composition and method of using same," Serial No. 216,098, filed June 27, 1938, in the United States 15 Patent Office.

In the invention just identified, I have proposed a composition which acts as a medium for effectively shutting off water in formation without appreciably affecting oil bearing sands. The 20 present invention is adapted to be utilized in an embodiment of the invention, after the material described in my first mentioned invention has been used.

An object of the present invention is to provide a composition which will effectively seal formation under adverse conditions. By adverse conditions, I mean a composition which is capable of setting and becoming water-resistant where the water is strongly alkaline or saline in nature, or where the water is hot. In fact, an object of the present invention is to provide a composition which will set in the majority of cases where cement slurry could not possibly set.

Another object is the provision of a composition 35 which will have an initial set within forty (40) minutes to two (2) hours. This initial set depends upon the depth to which the composition is to be pumped, and such well conditions as have to do with temperature and pressure. However, 40 knowing the conditions, the readiness to set is controlled by the initial viscosity of the composition to be used.

Another object is the provision of a composition which is water impervious from its initial 45 set.

Another object is the provision of a composition for use in wells which will have a definite hard set within eight (8) to sixteen (16) hours.

Another object is the provision of a composition 50 adapted to allow a well operator to resume drilling within a short period of time after casing has been landed. With respect to the last named object, it is ordinary practice in cementing operations to cement around a casing and then allow 55 the cement to harden around the casing for a number of days prior to resuming well drilling operation. The present invention overcomes this long delay in shutting down a well being drilled.

For the purpose of illustrating an embodiment 60 of the invention,

The figure is a vertical sectional view of a well hole containing the composition of this invention and likewise illustrating the method of shutting off water.

Referring to the drawing, I have shown a well 6 hole 1 within which is received a casing 2. Between the casing and the well hole, I have pumped a material 3 adapted to function in the capacity of a water shut off medium. Any usual or ordinary method whereby material may be pumped 10 from the surface of a well hole downwardly through the casing and upwardly between the casing and the formation may be utilized. I prefer to provide material for that designated as 3 of the character described in my copending application Serial No. 216,098. Specifically, in said copending application for patent, I combine the following ingredients with clay calculated on a dry basis:

|                               | Parts by weight |
|-------------------------------|-----------------|
| Clay                          | 20              |
| 24-hour cement                | 100             |
| Calcium chloride              | 10.5            |
| Unslaked lime                 | 11              |
| Prepared bentonite (para-gel) | 8               |
| Litharge                      | 25              |
| Flake caustic                 | .5              |
|                               | .05             |

In actual use and service, the clay is thoroughly mixed with water to the consistency of a jelly and the Stormer viscosity is in excess of 75 centipoises. For convenience, I term this material as composition #1.

The composition of the present invention, which I term composition #2, comprises the following

|                               | Parts by weight |
|-------------------------------|-----------------|
| Clay                          | 25              |
| Cement                        | 85 1/2          |
| Calcium chloride              | 11              |
| Unslaked lime                 | 8               |
| Prepared bentonite (para-gel) | 40              |
| Litharge                      | 8               |
|                               | 1/2             |

For a two (2) ton mix, the following proportions are utilized.

|                    | Pounds |
|--------------------|--------|
| 24 hour cement     | 45     |
| Calcium chloride   | 210    |
| Unslaked lime      | 220    |
| Prepared bentonite | 160    |
| Litharge           | 160    |
|                    | 10 50  |

Using the formula above set forth either for a two (2) ton mix or by parts, the said materials are thoroughly admixed in any well known manner and water added. For instance, assuming 55 the two (2) ton mix, the materials designated are thoroughly mixed with varying amounts of water, depending upon the initial viscosity of the liquid composition to be pumped into the well.

After thorough mixing, I add to the composition 60

750 pounds of clay and 2250 pounds of 24-hour cement, in dry form. The completed composition is now ready for use in a well hole.

I have found that the amount of water which must be added to the two (2) ton mix varies with the depth of the well hole. It has been found by graphic analysis that the number of barrels of water used with respect to the depth of hole is a straight line, and that if initially 2½ barrels of water to a two (2) ton mix is necessary for a 500 foot depth of hole, that for all other depths a straight line reading may be obtained, for instance:

2,000 feet depth 3 barrels of water; 3,500 feet depth 3.5 barrels of water; 8,000 feet depth 5 barrels of water; and so on.

The operation, uses and advantages of the composition just described, as well as its advantages with relation to composition #1, are as follows:

20 While I deem it preferable to use composition #1 in place of cement, still it is possible in the practice of the present invention to utilize cement slurry between the periphery of the casing and the wall of the hole. As is general practice, the casing carries at its lower end a shoe 4. This shoe is landed upon the formation and the casing may be filled with a definite quantity of composition #1 as indicated at 3. There is immediately pumped on top of composition #1 contained within said casing, a quantity of composition #2 indicated at 5. A frangible plug 6, of some type, to-wit, one which is easily breakable or may be drilled, such as a wooden plug, is then placed on top of composition #2, and the usual hydraulic means applied for forcing the plug and the two compositions downwardly within the casing. During this movement, the casing is constantly moved up and down slowly so as to prevent any freezing of the casing within the well hole and to assure that composition #1 is flowing properly between the periphery of the casing and the wall of the hole. The well operator readily determines from his pump the instant that the plug strikes the bottom of the well hole. When this occurs, the casing is landed so that the compositions cannot again enter the casing. Also, the water which is usually used for driving the plug may remain within the casing to prevent any upward movement of the plug. Composition #1 will remain in place and tend to shut off the water sands, although not appreciably affecting the oil sands. Composition #2 will form itself about the casing shoe and a portion of the casing and extend into the formation. After the compositions have been allowed to set for a given time, drilling of the well may proceed, if necessary, and to this end, a bit may be lowered within the casing to drill out the wooden plug or break up the frangible member. Further drilling of the well may continue, followed by the lowering of a liner within the casing, as is evident to any one skilled in this art.

As stated, I need not use composition #1, but composition #2 provides a rapid hardening wa-

ter-impervious material which may be placed around the casing and its shoe, to the end that a resumption of drilling operations, if necessary, may be had within a short period of time.

I claim:

1. A new composition of matter comprising the reaction product of relatively small amounts of clay, twenty-four hour cement, calcium chloride, unslaked lime, bentonite, lithage and water, and adding thereto relatively large amounts of dry powdered clay and dry powdered twenty-four hour cement, whereby the final composition of matter is of a pumpable fluid consistency having an initial setting period of from 40 to 120 minutes.

15 2. A new composition of matter comprising the reaction product consisting of 25 parts by weight of clay, 85½ parts by weight of twenty-four hour cement, 11 parts by weight of calcium chloride, 8 parts by weight of unslaked lime, 8 parts by weight of bentonite and ½ part by weight of lithage and water, admixed with 37.5 parts by weight of dry powdered clay and 112.5 parts by weight of dry powdered twenty-four hour cement, whereby the resultant product is of a pumpable fluid consistency having an initial setting period 25 of from 40 to 120 minutes.

3. The method of preparing a pumpable fluid composition product for use as a water shut-off in wells which comprises thoroughly admixing relatively small quantities of clay, twenty-four hour cement, calcium chloride, unslaked lime, bentonite and lithage with water to form a fluid reaction product, adding to such reaction product in dry form relatively large amounts of clay and twenty-four hour cement, and then admixing the mass into a homogeneous product.

35 4. The method of preparing a pumpable fluid composition product for use as a water shut-off in wells which comprises thoroughly admixing clay, twenty-four hour cement, calcium chloride, unslaked lime, prepared bentonite and lithage with a predetermined quantity of water, which quantity of water is determined by the depth of the well hole in which it is to be used, to form a fluid reaction product, adding to such reaction 35 product in dry form relatively large amounts of clay and twenty-four hour cement, and then admixing the mass into a homogeneous product.

45 5. The method of preparing a pumpable fluid composition product for use as a water shut-off in wells which comprises thoroughly admixing 50 25 parts by weight of clay, 85½ parts by weight of twenty-four hour cement, 11 parts by weight of calcium chloride, 8 parts by weight of unslaked lime, and ½ part by weight of lithage with 55 a predetermined quantity of water, which depends upon the depth of the well hole in which the product is to be pumped, to form a reaction product, adding to such reaction product in dry powdered form, 37.5 parts by weight of dry powdered clay, and 112.5 parts by weight of dry powdered twenty-four hour cement, and then admixing the mass into a homogeneous product.

VERN W. DAVID.